

July 27, 1943.

C. C. HERITAGE

2,325,055

THERMAL INSULATION

Filed May 22, 1940

2 Sheets-Sheet 1



Inventor  
Clark C. Heritage

by W. Bartlett Jones,  
Attorney.

July 27, 1943.

C. C. HERITAGE

2,325,055

THERMAL INSULATION

Filed May 22, 1940

2 Sheets-Sheet 2



Inventor  
Clark C. Heritage  
by W. Bartlett Jones  
Attorney.

Patented July 27, 1943

2,325,055

# UNITED STATES PATENT OFFICE

2,325,055

## THERMAL INSULATION

Clark C. Heritage, Cloquet, Minn., assignor to  
Wood Conversion Company, Cloquet, Minn., a  
corporation of Delaware

Application May 22, 1940, Serial No. 336,495

8 Claims. (Cl. 154—44)

The present invention relates to thermal insulation material, and more particularly to fiber masses and to insulation formed from such fiber masses into loosely felted masses such as are advantageous for thermal insulation and sound deadening.

The primary use of fibrous insulation is for thermal purposes, but it is also useful acoustically. The major characteristics of the fiber herein described are with reference to thermal uses, but some of the characteristics apply to the assembly of fibers into mats or masses, and more particularly to handling and to felting the fiber into spaces, independently of the use.

Heretofore, the applicant's assignee has provided a chemically-cooked vegetable fiber especially prepared for packaging into sealed slabs for thermal insulation of refrigerator cabinets. A special machine was provided for packing the fiber. Spafford U. S. Patent No. 2,073,655 describes the machine, its use, and to a degree, the fiber referred to. It is therein explained that the loosened fiber is dropped into a hopper to fall in front of a reciprocating ram. The ram forces it forward into a spout or nozzle of rectangular cross-section. This discharges a continuous rectangular bat which is somewhat elastic. The bat is fed endwise into a receiving bag which is thereafter to be sealed or closed to provide an insulating slab. The bat is a loosely felted structure subject to compression and to a "spring back" after release from compression. A length of freshly made bat which is longer than the slab when not compressed, is pushed into the bag endwise thereof, and the bag sealed over it. The immediately available elasticity causes the bat to press endwise on the bag and its other faces with a view to assuring a full bag and avoiding creation of void space by settling. However, it has now been discovered that this elasticity is not permanent, and that the customary initial degree of felting is not sufficient to saturate the capacity for felting with the result that the fiber may settle. One of the results which was for a long time incomprehensible, was

the loss of elasticity and eventual settling. This is now understood and the knowledge of it has lead to the present invention. Practice of the invention employs a system to evaluate the fiber, permitting the provision of fiber to meet desired objectives when used in accordance with the evaluation.

The above mentioned prior use is a good example of some requirements of bulk fiber for insulation and other uses. It must felt well and have high insulating value for a minimum of material. It must felt well to retain a packed formation. It must have elasticity and resistance to compression. For a pneumatic felting process it must have a moderately low resistance to felting, or in other words, felt easily. These properties are vital to packing bulk fiber into a permanent insulating form of predetermined density. These qualities of the mass call for fibers which per se are flexible and resilient, and which in a mass have suitable properties to form a permanent and thermally efficient felted mass. It is to be understood that many properties of bulk fiber are referred to a mass of the fibers, rather than to individual fibers, in spite of the fact that the properties of the mass arise in the individual fibers. A mass of fibers exhibits properties which depend on all the fibers of the mass and also upon the manner in which the fibers are associated. When the density of a heterogeneous mass of fibers is changed, the properties of the mass are changed, even though the properties of individual fibers are unchanged. It follows, therefore, that any one property taken for consideration is not absolute. For example, the thermal insulation value of one batch of fiber is dependent upon how it is assembled and at what density it is assembled.

It is also known as a result of experience in developing the present invention, that the properties of a fiber per se vary according to the kind of natural lignocellulose used, for example whether it be aspen or jack pine; vary with the treatment of the lignocellulose material before, during or after the defibering process, for exam-

ple the exposure to one or more of the following conditions: heat, water, moisture, chemicals; and vary with mechanical conditions encountered in defibering. In short, every variable which affects the fibers per se, has an effect on the mass properties of the fiber.

It is the general object of this invention to produce from lignocellulose as a raw material, a fibrous product which has properties inherent in the fibers per se, so combined and of such value, that they may be employed in controlled felting aggregates to give thermally efficient insulation, which is non-settling when no binder is used and the union in the mat is dependent upon the qualities of the mass as to felting and elasticity.

It is an object of the present invention to convert lignocellulose materials into a fibrous product having a predetermined combination of desirable qualities.

It is a particular object of the invention to regulate the fiberizing process to control the discharge thereof so as to give initially a high degree of the desired fiber size distribution.

It is an object of the invention to produce a low cost fibrous material suitable for efficient thermal insulation when placed in random arrangement at a predetermined density without the use of binders.

It is another object of the invention to produce fiber with a controlled resistance to felting forces, whereby it may be more economically assembled, particularly in pneumatic processes where the fiber is felted from suspension in a gas.

It is also an object to produce fiber of controlled utility for any use involving felted masses of controlled density with or without binder.

It is also an object of the invention to control the compressive properties of fiber, such as those later defined, and other measurable properties, and to vary the combinations of properties according to intended uses.

A particular object of the invention is to control some properties of the fiber by controlling particle size distribution of the fiber in forming the fiber.

Various other and ancillary objects and advantages of the invention will become apparent from the following description and explanation of the invention.

The invention is explained by reference to the accompanying drawings in which:

Fig. 1 is a plot of "free-footage" and thermal conductivity of a series of fibers.

Fig. 2 is a plot of "free-footage" and thermal conductivity of a more general relationship with the curve of Fig. 1 imposed upon it.

Fig. 3 is a chart of courses which fiber may take from a defibering process to a finished mat, which courses influence the properties of the fiber for felt formation, and also influence the properties of the mat.

Fig. 4 is a front view of apparatus for use in determining the coarseness modulus of fiber.

Fig. 5 is a side view of the apparatus of Fig. 4.

Figs. 6, 7 and 8 are respectively cross-sections of Fig. 4 on the lines 6-6, 7-7, and 8-8, showing the fiber-filtering means.

The processes of reducing wood or like lignocellulosic material to fiber are many and different. For the present invention a process is preferred which reduces the raw material to fiber with little waste as non-fibrous material, with a minimum of chemical change, and with substantially

no extraction of constituents. It is not indicated that the heat and steam effect no chemical change, but the absence of liquid water and of active cooking chemicals, and the short time, mitigate against chemical changes comparable to chemical cooking, or even water-softening steps. Use of water in a process extracts some material and alters others. In particular it gelatinizes cellulose material where frictional work is done on it in the presence of water. These and other changes in the substance of the fiber greatly alter the properties exerted by a felted aggregate of the fibers. Therefore, one important step in controlling properties is to minimize change in substance. Suitable processes are to be found in British Patent No. 15,105, of 1911, Asplund U. S. Patent No. 2,008,892, MacMillan U. S. Patents No. 1,344,180, No. 1,476,032 and No. 1,515,062, the Banbury apparatus (see Robinson No. 2,142,334, referring to Serial No. 101,014, filed September 16, 1936), the Respats apparatus of Respass No. 1,976,297, the explosion processes of the Masonite Corporation, Laurel, Mississippi, and others. Noting that the Asplund machine must be specially operated and controlled in order to produce fiber within the scope of the present invention, it is to be understood that this is likewise true of other machines and processes. The quicker the process, the less the change.

In one phase of the British patent process wood chips and steam are fed to rotary grinders, such as stones with spaced faces, between which the wood is reduced to fiber. In the Asplund process, the fiber is similarly ground, but with metal plates, in a heated gaseous atmosphere, such as of steam, above 212° F. and at a temperature where the wood or other lignocellulose is softened. The higher the temperature the softer the wood, and hence the process is more quickly carried out, and the wood more thoroughly defibered.

In these processes the size of the fiber produced is controllable in part by the spacing or other controls of the grinding elements, among other variables. Where a wide spacing of opposed disks is used, as in the Asplund machine, the product may be rigid slivers, such as ragged forms resembling in size a tooth-pick or a match. These are referred to as "slivers" and the range of size may be large. As the spacing is narrowed, the slivers are reduced in number, and flexible fiber bundles increase and may predominate. Bundles are natural aggregates of ultimate fibers which are not completely separated. They may be secured together at one end, at the middle, or overall, or have mixed relations. Many bundles are found which are frayed at an end like a broom, presenting single or a few joined ultimate fibers. From two to several hundred ultimate fibers may constitute a "fiber bundle" as it is here defined for the purposes of the present invention. It is also to be understood that a sliver which is rigid may be fractured or bruised so that it is flexible to be considered herein as a bundle.

When the spacing of the grinding elements is made still closer, the bundles become less, slivers may disappear entirely, and ultimate fibers increase. As the setting may be made still closer to decrease bundles, there is danger of destroying some of the ultimate fibers, producing broken ones, called "fines" or "shorts," and even granular particles. The latter also may be present from bark in the raw material or from breaking off non-fibrous material which lies naturally between fibers.

The grinding process is capable of producing glivers, bundles, ultimate fiber, fines, and dust. By adjusting the machine the predominance of a certain type may be made to prevail. A substantially completely fibrous product may be taken from the machine with many of the permitted adjustments. The present invention permits control of variables to produce a product having controlled properties in a proper combination of such properties for selected uses.

To practice the present invention, it is first desirable to analyze the fiber by dividing it into fractions of predetermined sizes to determine a definitive coarseness modulus. From information thus obtained it may be predetermined what adjustment of the machine will deliver a product within a selected range of coarseness modulus, the whole of which product may be most efficiently used as bulk fiber useful for insulation. By such means a bulk fiber may be obtained meeting predetermined specifications.

The information obtained from use of one kind of raw material does not necessarily dictate the same operating practice and results for another kind or another species of the same kind. Properties of the mass derive in part from properties of the fiber, and these vary with the source of raw material. Nevertheless, the general procedure for practice of the invention is the same. It is, therefore, not considered necessary to give duplicative disclosures for several materials. To explain generally, it is stated that suitable fibers derived from aspen have a range of coarseness modulus from 60 to 160, while for jack pine the range is from 130 to 250. Nevertheless, certain other properties may be identical. In order to illustrate the invention, a discussion of the procedure is given with reference to jack pine, reduced to chips, and treated to the action of an Asplund machine in steam at a temperature of around 365° F. (150 lbs. gauge pressure).

The chips, particularly of old wood, are wet slightly with water so that they are more moist than air-dry, thus to prevent burning in the machine. Green wood is sufficiently moist for use without adding moisture. It may be mentioned that control of moisture at this point is one variable for effecting property-value control. The chips in the machine are heated, ground and may be discharged from the machine in about 45 to 70 seconds, more or less. The rate of production is another control variable. The discharge may have from about 50% to 150% moisture on the dry wood basis. The material is preferably dried directly without immersion in water. Water treatment is another control variable.

A result of direct drying is the inclusion of fines and dust. These may be eliminated by taking up in water, filtering, and preserving the large sizes. This adds to the cost by the extra drying which must follow. It also removes water-soluble material. Also under some conditions the drying after contact with water tends to lay down ends of fibers in bundles, or bundles or fibers cling together as agglomerate masses, and alter the insulation value. Therefore, for the tests herein reported, the material has not been immersed and then dried, but dried directly, unless otherwise specified.

The fines and dust are undesired in bulk fiber for insulation, for reasons discussed later. In handling, for example, these escape and may fill the air. By adding a bonding agent to the chips

or other form of raw material entering the machine, the dust and fines may be anchored to large particles. Rubber latex or other treating agents may be so used, as described in my copending application U. S. Serial No. 334,761, filed May 13, 1940, and Serial No. 336,577, filed May 22, 1940.

The use of a treating agent must be considered as a factor changing the character of the fiber. It has been determined that where the same wood is processed to a fiber and the fractions tested, there is a great difference in measured properties where the only processing difference is the use of a treating agent. The untreated and treated fiber may have the same coarseness modulus, yet be radically different in one or more measured properties. Various treating agents as follows have been used, such as rubber latex, paraffin wax, asphalt, montan wax, and rosin. Also there may be used fire-proofing agents, mold-preventatives and other agents. Of these rubber latex is preferred to minimize dustiness. It gives the fiber other desirable properties for felting into insulation mats. Fire-proofing agents, mold-preventing agents and other materials have been used with latex, as well as combination of material.

In proceeding to test the properties of the fiber discharged from the machine under the specific conditions above described, the machine was differently controlled in a series of runs, producing a relatively fine product in run No. 1, and a relatively coarse product in run No. 8, with gradation in between. The "particle size distribution" of each run was determined and expressed numerically on some selected but arbitrary standard. The one specifically referred to at this time results in a value reported herein as coarseness modulus.

#### DETERMINATION OF COARSENESS MODULUS

The principle employed involves a standardized screening of the material through a series of graded perforated plates, or screens, or both, of successive fineness, whereby a fraction No. 1 of coarse material is obtained, followed by fractions of successively finer material. There are numerous classification apparatuses available for such operations using fixed procedures. Some operate wet, some dry, and some by air. The present results were obtained on a wet classifier herein referred to as the "Laurel classifier" (Shop Order No. 4336) provided by the Machine and Foundry Company, Laurel, Mississippi. It provides first and second plates with drilled holes, and then two wire screens.

The classification results are expressed as follows:

| 60     | Fraction No.—    | Retained by              |
|--------|------------------|--------------------------|
| 1..... |                  | 1/16 inch drilled holes. |
| 2..... |                  | 3/64 inch drilled holes. |
| 3..... |                  | 32 mesh screen.          |
| 4..... |                  | 80 mesh screen.          |
| 65     | P-4 (past No. 4) | Passes 80 mesh.          |

The weight of each fraction is expressed as percent by weight of the total amount tested (all on dry weight bases). The "coarseness modulus" is obtained by adding:

- 4 × percent of fraction No. 1
- 3 × percent of fraction No. 2
- 2 × percent of fraction No. 3
- 1 × percent of fraction No. 4

giving total of (a number) which is the coarseness modulus, frequently referred to as C. M. This is a standard method of weighting results.

A full description of the classifier and of its operation is given later in the specification.

In Table I, the data and the corresponding coarseness modulus of the jack pine fiber are given for said runs No. 1 to 8, for which the machine setting was recorded, and is arbitrarily represented herein by the "Run No."

Table I

TABULATING PERCENT BY WEIGHT AGAINST FRACTIONS AND CORRESPONDING PROPERTIES

|                                    | Run. No.— |       |       |       |       |       |       |       |
|------------------------------------|-----------|-------|-------|-------|-------|-------|-------|-------|
|                                    | 1         | 2     | 3     | 4     | 5     | 6     | 7     | 8     |
| Fraction No.—                      |           |       |       |       |       |       |       |       |
| 1                                  | 1.0       | 4.4   | 8.2   | 19.0  | 32.4  | 39.6  | 49.6  | 53.8  |
| 2                                  | 4.2       | 6.8   | 10.6  | 13.4  | 11.8  | 10.8  | 8.8   | 7.6   |
| 3                                  | 42.0      | 40.2  | 33.2  | 27.8  | 21.0  | 21.4  | 17.8  | 16.8  |
| 4                                  | 29.8      | 27.8  | 29.2  | 24.0  | 21.6  | 16.2  | 12.8  | 11.0  |
| Past 4th                           | 22.4      | 20.8  | 18.8  | 15.8  | 13.2  | 12.2  | 11.0  | 10.8  |
| Coarseness modulus                 | 131.6     | 146.2 | 160.2 | 196.8 | 228.6 | 249.8 | 273.2 | 292.6 |
| "K" value                          | 231       | 239   | 235   | 239   | 238   | 249   | 257   | 257   |
| Free footage                       | 8.64      | 8.16  | 8.9   | 9.95  | 8.15  | 6.76  | 6.5   | 5.8   |
| Specific elasticity K <sub>E</sub> | 118       | 75    | 82    | 84.5  | 67    | 53    | 38    | 24    |
| Absolute elasticity M <sub>E</sub> | 373       | 399   | 331   | 341   | 363   | 478   | 478   | .517  |
| Specific felting K <sub>F</sub>    | 82        | 65    | 78    | 29.5  | 18    | 11    | 8     | 0     |
| Absolute felting M <sub>F</sub>    | 347       | 358   | 327   | 263   | 260   | 281   | 271   | 0     |

Table I also gives the insulation value (K-value) of the fiber measured at 3.8 pounds per cu. ft. density, which corresponds to the "footage" of 3.15 board feet per pound. This footage is the one chosen in the testing procedure for the "specific" values K<sub>E</sub> and K<sub>F</sub> used herein. The given "K" value represents heat transmission in B. t. u., per sq. ft., per 1-inch of thickness, per 1° F. temperature differential, per hour, when the test is made on a sample of 1-inch thickness with the fiber in direct contact with the hot and cold plates, and is a standard unit well known in the art. The table also gives "free-footage," which represents an extrapolated hypothetical state where the fiber is unfelted except by the force of gravity. In plainer words, it represents the "fluffiness" of the fiber, and is mathematically expressed as a volume per unit-weight, or board feet (12 x 12 x 1 inches) per pound. It is a very useful and easily measurable property of fiber explained more in full herein-after, which explanation includes reference to the remaining properties listed in Table I.

A single value of coarseness modulus theoretically corresponds to a variety of combinations of fractions. Considered only mathematically, it is not a true indication of the distribution of fractions. But practically, it is significant when the fibers of different coarseness modulus are being compared, if the fibers are produced by the same conditions, as for example by the same machine. The distribution is an average result of all the conditions. Considered mathematically, the said average is the average of the probabilities. The same machine, or the same process tends to present the same probabilities when the conditions are the same, and to vary from sameness in a regular way related to changing conditions. Accordingly, the coarseness modulus is an indication of both changed conditions and changed result, and is a comparable value.

The higher the coarseness modulus, the more coarse the fiber mass will be.

From wood, the mass may have slivers, bundles,

ultimate fibers, and fines (broken fibers or particles not fibrous). It has been found that slivers in the mass lower the insulating efficiency. Increasing coarseness modulus shows an increasing content of slivers, and of itself at the high end indicates lowered thermal efficiency for insulation.

On the other hand, ultimate fibers favor insulating efficiency, and decreasing coarseness modulus indicates increasing content of ultimate fibers, and high thermal efficiency. It follows that 100% ultimate fibers is the optimum to be desired. However, other properties and other considerations enter the picture. A mechanical defibering action cannot readily be carried out to produce 100% ultimate fibers. As the process is adjusted to eliminate slivers and bundles and increase ultimate fibers, some ultimate fibers are broken to make dust and fines. The process may be adjusted to produce mixtures exhibiting a desirable combination of fiber sizes, and the coarseness modulus is a simple key for production control.

The matter of handling fiber masses, in baling, shipping, forming mats, felting, and the like, is related to the so-called "dustiness" of the fiber mass. For the purposes of description "dustiness" or "flying dust" of a mass of fibers, is the content which can leave a felted matrix of the fiber mass and appear as "dust" in the air. Ultimate fibers may constitute part of this dust. For commercial purposes dustiness is undesired. Ultimate fibers may appear as flying dust from a matrix which is largely coarser fibers, which matrix acts like a screen with large openings predetermined by the general coarseness of the fibers. Consequently, although the presence of ultimate fibers in a mass of fibers generally much coarser, is desirable as adding to the insulating efficiency, it may be undesirable as creating dustiness. If the matrix in general were ultimate fibers the screen-effect of the matrix would be finer and ultimate fibers would not appear as dust.

It follows, therefore, that in converting wood or the like to bulk insulating fiber, without loss of a portion, or addition thereto to control the properties, it is very important to avoid a high percentage of coarse, and also to avoid a high percentage of fine where there is considerable of coarser material. The present invention permits the defibering of wood or the like to be controlled to yield a total product falling within a given range of particle size distribution, in order to secure a high degree of practical utility commensurate with a high degree of insulation efficiency.

With respect to the Asplund machine operating on lignocellulose materials, such as wood, the invention contemplates adjusting the machine to yield a total product falling with a range of coarseness modulus. Therefore, the thermal conductivity is not the sole criterion on which to base the desirability of the fiber. However, it is significant to check the fiber chosen for other desirable characteristics.

The coarseness modulus referred to in this description is a convenient index for particle size distribution. It is specific for the classification system employed, and that is arbitrary and in practice not a universally accepted standard. However, one system may be converted fairly accurately to another, using the known laws governing particle size distribution. Fiber masses

with the same coarseness modulus may vary in important mass properties.

There is another property of fiber masses which appears to be an aggregative property, comprehending other properties, such as the elasticity of the fibers per se, and the felting characteristics of the fiber. Reference is made to the application of Anway U. S. Serial No. 313,920, filed January 15, 1940, which discusses means and methods for determining the so-called "compressive properties" of fiber masses. "Free footage" is one of the compressive properties and is the preferred term for the said aggregative property. It is defined in terms of a density-factor of a fiber mass at zero compression. Actually, the "free footage" is the reciprocal of density, and is given in units of board feet per pound of fiber, a board foot being  $12 \times 12 \times 1$  inches. The value is one obtained by extrapolation by the procedure of the below-quoted paragraphs. These paragraphs are quoted from said Anway U. S. Serial No. 313,920, filed January 15, 1940, and are sufficient herein to give the full procedure for determining the compressive properties, including free-footage.

#### "PRACTICAL PROCEDURE

"Place 158 grams of loosened fiber in a cylinder of 8-inches diameter and 22 grams of the same loosened fiber in a 3-inch diameter cylinder presenting the same character of interior surface. Place the cylinder on a platform scale adjusted to read zero (or else the weight of the fiber, the difference being negligible). With a flat plate compress the large column of fiber at the rate of 1 inch in 32.4 seconds until it is 2 inches high (a reciprocal density of 2 board-feet per pound). Record the pressure on the scale as reading  $P$  pounds, and the corresponding height of the column, at approximately each half-inch of advance, or a sufficient number of observations to locate a mean straight line. Record the final pressure  $Q$  at column height of 2 inches. Upon attaining said last mentioned height, immediately remove the plate to release the column. Measure the height (board-feet per pound) attained by the column after such spring-back, and record as  $H$  inches (or board-feet per pound).

"Then substitute the smaller cylinder, and compress at the same rate until the column height is 2 inches (board-feet per pound), and record the pressure as  $R$  pounds.

"The following data are thus obtained:

Table IV

| Board-feet per pound or "footage" | Footage on 8-inch spring-back | 8-inch column         | 3-inch column |
|-----------------------------------|-------------------------------|-----------------------|---------------|
| 2.<br>(The series)                | H.<br>(The series P.)         | Q.<br>(The series P.) | R.            |

"Select semi-log graph paper having a log scale vertically beginning at log of 1, (which is zero), and mark equal divisions of 'footage' units horizontally. On the chart, plot the series of observations using  $P \times 2.86$  and the point: 2 footage and  $Q \times 2.86$ . Draw a mean straight line through these points. Where the line cuts the bottom of the chart (at 1), designate the point and the reading as 'free footage.' Label the straight line 'C-line,' or 'compression line.'

"From footage  $H$  on the C-line draw a horizontal line to a point of intersection with the line for footage 2. Draw a straight line from this

point to the 'free-footage' and label the line 'Cs-line,' or 'spring-back line.' Draw a vertical line at  $H$  footage and label 'sprung-back footage.' On the latter line, subtract the ordinate values of the intercepts with the C-line and Cs-line, and record the difference. Mark this difference on the log scale as a point on the H-footage line, draw a straight line from the point to the 'free footage' point, and label 'Ke-line.' Take any two points on the Ke-line. Subtract the ordinate values (the log units, not the pounds) and divide the difference by the difference of the free-footage values. Neglect the minus sign and record the value as  $Mr$  or the 'Absolute elasticity.' Draw a vertical line through 3.15 footage and mark 'specific footage.' At the intercept of the Ke-line and the specific-footage line, record the force value as the 'specific elasticity.'

20 "Using the formula (wherein for the large cylinder  $y = \text{friction at 2 board-feet}$ )

$$y = 2.86 (4.269R - .6Q)$$

25 solve for  $y$ . Using the formula (wherein  $K = \text{coefficient of friction}$ )

$$K = \frac{8.538R - 1.2Q}{3.2Q - 8.538R}$$

30 solve for the value  $K$ .

35 "On the vertical line for footage of 2, plot the value of  $y$ , and draw a straight line to the free footage, marking the line 'friction line.' On the friction line at H-footage record the force value as a 'deduction' value. On the C-line at H-footage read the force value, subtract from it the said deduction value, and record the difference as 'felting at 2 board-feet.' Plot this felting value on the vertical line for 2 board-feet, connect the point by a straight line with the free-footage point, and label the line 'Kf-line' or 'felting line.' Determine the slope of the Kf-line by dividing the difference in ordinate values (the log units, not the pounds) of two selected points in it by the difference in footage values of said two points, and label the figure so obtained with or without the minus sign as 'absolute felting' or 'Mr.' At the specific-footage on the Kf-line record the force value as 'specific felting.' Thus the values determined are compressive properties, listed in Table V.

Table V

| 55                              | Absolute values | Specific values (at 3.15 footage) |
|---------------------------------|-----------------|-----------------------------------|
| Free footage                    |                 |                                   |
| Absolute elasticity ( $Mr$ )    |                 | Specific elasticity ( $Ke$ )      |
| Absolute felting ( $Mr$ )       |                 | Specific felting ( $Kf$ )         |
| Coefficient of friction ( $K$ ) |                 |                                   |

60 65 On the lines: C-line, Cs-line by projecting horizontally to the C-line, Ke-line, friction line, Kf-line, may be read for any selected footage the following values, respectively: pounds per sq. ft. in compressing, the spring-back height obtainable at any time on releasing during the compression, pounds per sq. ft. exerted by elasticity at any point in the compression, pounds per sq. ft. used in overcoming friction while compressing, and pounds per sq. ft. used in producing felting at any point in the compression."

70 75 "Impact resistance" is another important property related to the compressive properties. It may be determined as described in Anway U. S.

Serial No. 313,919, filed January 15, 1940. Briefly, explained, a vertically axial container, carrying a column of fiber to be tested is dropped repeatedly to give an impact of 1 foot-pound on the column. The fiber thus acquires a constant density or volume. The density, expressed as its reciprocal in board feet per pound of fiber at 1 foot-pound impact is the impact resistance adopted for comparisons of fiber.

The impact resistance in foot-pounds is but another manifestation of elasticity of a felted fiber mass. Whereas the specific elasticity is measured at 3.15 board feet per pound, the impact resistance is related to that density when expanded which just resists settling at 1 foot-pound impact. A mathematical relation between specific elasticity and "impact resistance" is more complicated than saying they are the same thing, recognizing, however, that they arise from the same characteristics of the fiber. It has been determined that where a mass is self-felted for insulation mats to a density at least equal to the tested "impact resistance" as defined, the mat is sufficiently non-settling for use in refrigerators and like places where substantial shock in daily use, as in closing a refrigerator door, is encountered.

Hundreds of determinations of the properties of fiber by the above compressive and impact procedures evidence their real values in evaluating fibers. Hundreds of determinations of coarseness modulus for the evaluated fibers show its reliability for control of fiber, especially in producing it, to give the desired evaluations. These evaluations permit the setting of limits for the coarseness modulus for the present invention.

A fiber mass may be characterized in part by its coarseness modulus, which gives very definite information about the physical size of the components of the mass. It is a property which can be readily measured, and which is not altered except by some destructive action changing the sizes of particles. It is independent of changes within the fibers per se.

Free-footage, on the other hand, is not such an independent single property. It is determined in part by intrinsic qualities of individual fibers, and also in part by the coarseness modulus. However, it eliminates the state of aggregation. Free-footage must be determined on fibers in a mass which is substantially unfelted. A mass of fibers which has been felted must be unfelted to determine its free-footage, and both acts may be so severe as to break fibers, thus changing both the coarseness modulus and the free footage. Therefore, in unfelting fibers to determine free-footage, care should be exercised not to break fibers.

For a given kind of fiber having the same general history but differing in coarseness modulus, there is a general correlation between coarseness modulus and free-footage. However, for different types of fiber, the same correlation does not hold. Accordingly, for fibers of the same type, comparisons may be made by reference to coarseness modulus. For fibers varying in type, comparisons may be made by reference to free-footage or to both free-footage and coarseness modulus. For example, it has been found that the thermal conductivity of many fibers, untreated, and treated, fractions, and mixtures of fractions, are correlatable with free footage.

When lignocellulose is defibered in an Asplund machine, treating agents may be added as set forth in Asplund No. 2,047,170. Rubber, such as

70 latex, is a treating agent described in my co-pending application, U. S. Serial No. 336,577, filed May 22, 1940, as a particularly valuable one to minimize dust in bulk fiber, and to improve

5 the properties for certain insulation applications.

Bituminous substances, such as petroleum asphalt, is another type of treating agent, described in my copending application, U. S. Serial No. 334,761, filed May 13, 1940. These agents 10 weight the fibers, and two masses which are respectively treated and untreated, may have the same coarseness modulus, but different free-footage values.

Plotting the values given in Table I of 15 free footage and coarseness modulus, or the "k-values" and coarseness modulus, gives correlations less perfect than that obtained by plotting "k-value" against free-footage. This is in agreement with much other experience, 20 namely that free-footage correlates "k-values" very well for miscellaneous varieties of fibers, as shown in the said Anway application U. S. Serial No. 313,920, filed January 15, 1940.

In Fig. 1 hereof, the series of Table I is plotted 25 with "k-value" of interfelted fiber mats lacking adhesive on the vertical axis 10, and free-footage on the axis 11, giving the straight line correlation 12. This is in agreement with Fig. 2 hereof which is Fig. 17, of Anway application U. S. Serial No. 313,920, filed January 15, 1940.

Fig. 2 has thermal conductivity (measured at 3.8 pounds per cu. ft.) of numerous interfelted mats of fiber lacking adhesive, on the axis 13, and free footage of the same fiber on the axis 14.

30 The band area 15 defined by the straight lines 16 and 17 was produced by plotting on this graph 48 samples of wood fiber having irregular variations in particle size distribution, with and without treating agents, and drawing lines bounding the average area determined by the specific plots. 75% of the points plotted lie within the band.

The values of line 12 in Fig. 1 have been transferred to Fig. 2 as line 18 thereon, in confirmation of the fact that the specific runs of 45 Table I, fall within a more general relation covering greatly different conditions. Neither the band of Fig. 2, nor the line 12 of Fig. 1 are given herein as a criterion for other fibers, but only in 50 illustrations of the general tendencies of the relationships, and of the value of the control and evaluation procedures.

With respect to the value of free-footage, it 55 is to be understood that it is a value dependent on the fibers being completely free and unfelted by an applied force of compression. If the fibers are felted by compression, or by immersion in water, filtering and drying, the so-called free-footage determined on such partially felted fibers is not the true free-footage. Thus, for 60 example, dry unfelted fiber which is baled, then broken, must be completely loosened from the felted relation produced by baling, before the true free-footage may be determined. This may be done for test purposes by suction apparatus, or adequate picking means, so used as not to introduce felting, and to avoid breaking fibers.

70 One of the characteristics of the Asplund machine is, that it discharges moist fiber in a loose substantially unfelted condition, which may be easily and directly dried. In fact the steam pressure at discharge from the machine may be used to convey the fiber in a conduit to a conveyor belt of a drier, without thereby subjecting

it to a felting compression which destroys its substantially unfelted form in which the free-footage may be immediately determined. Avoidance of wetting the fiber to the point of matting, and avoidance of suspending it in water, are both economically important where a free-footage value is sought, for two major reasons. The wetting produces clotting, which requires unfelting, with possible injury or breaking of the fiber. Immersion in water and filtering, in addition to the above, dissolves solid matter from the fiber with economic loss. It has other effects which change the physical properties of the fiber, such as the felting and elastic characteristics, thermal conductivity and free-footage. Thus, it may be resorted to where a desirable change may be effected.

However, where controlled coarseness modulus is sought, the clotting of the fiber by water is not a serious interfering matter. The clots may be unfelted in water in which the fiber may be present for determining the coarseness modulus as later described. Accordingly, when fibers are to be characterized by coarseness modulus, the fiber, as discharged from an Asplund machine or the like, may be wet and clotted, or merely moist, and either form may be dried directly, or further wetted or suspended in water, recovered and dried.

Where the fiber is to be characterized by free-footage, it is preferred that the fiber be formed in the absence of suspending or clotting water, and that it be dried directly from its original condition. These make unnecessary any effort to un-felt it for the purpose of evaluation. Such preferred procedure preserves all the solid substance of the vegetable matter from which it is derived.

Not all the fiber masses made by direct drying or otherwise as herein referred to, are efficient for insulation purposes. A large amount of slivers gives high coarseness modulus, lower free-footage, and poorer insulation efficiency. To avoid too much of the fines and dust, the product must be made with a permissible coarseness, and a small amount of slivers may be tolerated. It has been found that when the fresh directly dried fiber has a free-footage in excess of 6.0, it is satisfactorily efficient for handling, baling, loosening, and packing into insulating spaces, with the proviso that where natural felting without adhesive is used, it has also other required properties. It is likewise satisfactory for building up flexible blankets, with adhesive or without it. Where a water-adhesive is used, the fiber need not be dried, except to determine free-footage. The moist fiber may be directly conveyed to forming machines where it is built up in the presence of adhesive to provide a mat. Where adhesive is used as a binder for the fibers in the mat, certain qualities may be neglected.

For the purposes merely of insulation the fibers may be made without slivers with lower coarseness modulus. However, fines and broken fibers tend to increase, giving dustiness, and also lowered insulation value. Practically, therefore there is a range for coarseness modulus wherein the fibers as a whole product of lignocellulose, are valuable as bulk fiber for insulation. The various kinds of lignocellulose may have individual ranges within the broader general range. Aspen is typical of the short-fibered woods, and jack pine is typical of the long-fibered woods. Therefore, the range for

aspen more or less lies at one end of the general range, while the range for jack pine lies at the other end. From experience with many samples of fiber made in the Asplund machine, a coarseness modulus from 60 to 250 is the general range which is practically useful and efficient. Aspen has the range 60 to 160, while Jack pine has the range from 130 to 250.

The free-footage value determined after direct drying runs generally from 7 to 12, but sometimes higher and lower values are encountered. This includes fiber with and without chemical treatment.

The process is preferably carried out in the Asplund machine by introducing moist or slightly wetted wood chips into a chamber within which is a steam pressure of 150 pounds per sq. inch, or a temperature of 365° F. This is not a critical pressure, nor is the steam temperature an indication of the actual temperature of the wood while being reduced to fiber. The important points in the process, are the absence of water to suspend the fibers, the action of heat in softening the wood, and the quick action. The free-footage of the resulting fiber is dependent upon the setting and operation of the machine, in a complex relationship, which can be best determined by empirical tests, comparing results to operating conditions. The series in Table I is representative of changes in the product resulting from adjustment of grinding elements. In many months of controlling Asplund machines, the coarseness modulus has been used to regulate the machine to control the product. At the same time the compressive properties (including free-footage) and the impact resistance test have been used to evaluate the fibers.

With guiding experience, a selected range of coarseness modulus practically assures that the fiber falls within the useful range of desired properties, and the evaluation tests point out what the specific properties actually are. In several hundreds of determinations, the coarseness modulus has thus been shown to be a reliable index to the suitability of the fiber for thermal insulation and the handling thereof to produce it.

Although the foregoing has referred to raw wood as the original material, this is largely because of more experience with it. In practice it is an economic raw material. However, the same process has been applied to chips which have been softened by chemical cooking and washed. It has been practiced on chips fed to the Asplund machine with cooking chemicals in solution, such as caustic soda, monosodium sulfite and others. It has been operated upon mixtures of raw chips and cooked chips, and mixtures of raw chips and both wet and dried pulp-mill screenings, from both sulfite, soda, kraft sulfate and monosulfite cooking processes. Accordingly, the term "lignocellulose" as used herein, contemplates such mixtures and modified forms.

Where the fiber is to be dry-felted, using the inherent felting qualities of the mass of fiber, the felting and elasticity properties, as determined by the compressive procedure, are very important controls. These are related to the formation of efficient mats which do not settle and which may exhibit an elasticity in the mat. But where the fiber in the mat is bound with an adhesive, the mat is more stabilized against settling, and the felting and elastic properties are not essential controls. The free-footage how-

ever, considered as a measure of the fluffiness of the fiber is an important control. Also the coarseness modulus remains as an important control. These properties, as controls, may be better explained by reference to hypothetical cases. First, consider that rigid fiber-like material such as wire or extruded plastics, with smooth side walls, like little rods, are assembled in a mass which will give a coarseness modulus. These will exhibit little fluffiness and will pack like nails in a barrel. Then consider the same sizes of material which is like the wood fiber here described with frayed ends, as in bundles, with elasticity, with flexibility and with bent, curved or other non-linear particle forms. These will pack with greater volume than the rod-like forms. This difference is indicated by the free-footage value.

Examination of the "compression-line" of the above described compression test procedure, will show clearly that the free-footage value is not dependent upon the action of the fiber under compression (even though it is so determined), as are the elastic and felting properties. It follows, therefore that the elimination of the characteristics of felting and elasticity from the broader definition of the fiber of the present invention is justified by experience, by hypothetical considerations, and by a test procedure and the mathematical analysis of the results of such procedure.

For the working of bulk fiber to produce self-felted (without binder) insulation mats of the desired character, individual properties of the fiber mass have significance. The specific felting value  $K_F$  must not be too high, or a well felted self-supporting mat, as in a refrigerator cabinet, cannot be obtained. On the other hand, the specific elasticity value  $K_E$  cannot be too low, or a felt resistant to settling cannot be obtained. The desired thermal effect or  $K$ -value imposes an upper limit on C. M. Settling imposes a lower limit on  $K_E$ , which in turn imposes an upper limit on C. M. Ease of felting imposes an upper limit on  $K_F$ , which in turn imposes a lower limit on C. M. Adequacy of felting imposes a lower limit to  $K_F$ , which in turn imposes an upper limit on C. M.

As a result, the suitable self-felting fiber may be characterized as having a range for coarseness modulus, a range for specific felting, a minimum limit for free-footage, and a minimum limit for specific elasticity. Collateral and subsidiary properties may be added, which flow from those specified. Thus, for example, the absolute elasticity may have a lower limit. A self-felting fiber mass within the present invention must therefore have:

|                           |            |
|---------------------------|------------|
| Coarseness modulus        | 60 to 250  |
| Free-footage              | 6 or more  |
| Specific felting $K_F$    | 20 to 80   |
| Specific elasticity $K_E$ | 50 or more |

Additionally, for efficient insulation a felt which is resistant to settling, and which has a density of 3.15 board feet per pound, must have a  $K$ -value not over .25. The numerous limits above relate to the working qualities of the fiber to produce a mat of such  $K$ -value. Where the term "resistant to settling" is herein employed, it means with respect to repeated impacts of not more than one foot-pound.

As explained these are interrelated and dependent properties, no one of which predetermines one other. The defibering machine may

be operated in an ordinary manner at one time to produce fibers within the above, and at another time to produce fibers outside the above. Treatments of such fibers may change properties within the above to properties outside the above, and vice versa.

Many conditions not referred to above affect the results. For example, Table I was the result of operating one size of Asplund machine. A 10 different size of such machine gives a different distribution of the C. M. determinant fractions, and hence different properties. Thus fibers from said two machines, having the same C. M. may have quite different properties. Table II shows 15 Jack pine fiber made on a machine of size different from the machine used to make the fibers of Table I.

Table II

|                           | Sample S-218— |      |      |      |      |
|---------------------------|---------------|------|------|------|------|
|                           | 28            | 24   | 27   | 23   | 26   |
| 25 C. M. fraction No.—    |               |      |      |      |      |
| 1                         | 2.4           | 5.0  | 6.0  | 10.0 | 14.4 |
| 2                         | 28.4          | 15.6 | 24.8 | 18.8 | 20.4 |
| 3                         | 18.2          | 31.2 | 24.8 | 24.8 | 25.4 |
| 4                         | 28.2          | 31.0 | 27.0 | 30.2 | 23.2 |
| P4                        | 22.8          | 17.2 | 17.0 | 15.7 | 16.6 |
| Coarseness modulus        | 159           | 160  | 175  | 176  | 193  |
| 30 Free footage           | 10.2          | 9.2  | 9.5  | 9.7  | 8.9  |
| Specific elasticity $K_E$ | 147           | 115  | 145  | 90   | 110  |
| Absolute elasticity $M_E$ | .31           | .34  | .34  | .31  | .34  |
| Specific felting $K_F$    | .62           | .33  | .43  | .40  | .27  |
| Absolute felting $M_F$    | .26           | .25  | .26  | .24  | .24  |
| "K"-value                 | .227          | —    | .220 | .232 | —    |

In the above table, sample S-218-28 is only a fairly satisfactory self-felting bulk fiber, since its  $K_F$  value is toward the top of the range. It is more resistant to felting forces. Even though its 40 C. M. is within the range for jack pine, it is near the low end and this indicates a danger that the fiber may not evaluate as satisfactory. It may be observed that as the C. M. goes up, the  $K_F$  goes down. However, such fiber is more satisfactory 45 for making adhesively bound felted mats, where self-felting is not so important.

In Table I, an examination of the fibers in the light of the limitations placed on them by the present invention for self-felting purposes, indicates that only runs Nos. 2, 3 and 4 provided the proper fiber. The  $K_F$  values of the others are outside the range 20 to 80. Run No. 8 is also not a suitable self-felting fiber because of low free-footage, and runs No. 7 and 8 are also out on account of low  $K_E$ . Run No. 1 is out on account 55 of high  $K_F$ . It is to be noted that although excluded run No. 1 of Table I has a  $K$ -value below .25, the fiber does not produce the physical properties for the most desirable mat.

Run No. 4 of Table I is comparable to S-218-26 of Table II on coarseness modulus, and shows a wide variation in  $K_E$ . Conditions within the different sizes of machines and their operations, are thus reflected in difference in properties for fiber of substantially the same C. M.

However, for fiber to be bound adhesively into an insulating mat, only the coarseness modulus and free-footage are essential determinants, and on this basis in Table I, the fiber of runs Nos. 1 to 6 are suitable. Runs Nos. 7 and 8 are excluded as having a C. M. over 250, and run No. 8 is excluded as having a free-footage below 6. It will be observed that these are also less efficient insulators, than runs Nos. 1 to 6.

The following table gives a number of fiber evaluations, and indicates treatments. Recovery is exemplified at 38 by the term "filter." The recovered fiber may be dried in any form at

Table III (rough jack pine)

| Treatment                                                       | None   |        |                 | Rubber solids<br>(1% on fiber) |        |        | Asphalt |                |                 | Chemical |
|-----------------------------------------------------------------|--------|--------|-----------------|--------------------------------|--------|--------|---------|----------------|-----------------|----------|
|                                                                 | Item 1 | Item 2 | Item 3          | Item 4                         | Item 5 | Item 6 | Item 7  | Item 8         | Item 9          | Item 10  |
| C. M.                                                           | 131.6  | 196.8  | 292.6           | 132                            | 204    | 254.4  | 242     | 252            | 311             | 229      |
| K-value                                                         | .231   | .239   | .257            |                                |        |        | .238    | .237           | .249            | .262     |
| M.E.                                                            | .373   | .341   | .517            | .422                           | .324   | .441   | .490    | .495           | .624            | .40      |
| M.F.                                                            | .347   | .293   | .0              | .326                           | .25    | .273   | .255    | .326           | .420            | .29      |
| K.E.                                                            | 118    | 84.5   | .24             | 98.5                           | 114    | 133.1  | 99.3    | .66            | 15.3            | 196      |
| K.F.                                                            | 82     | 29.5   | .0              | 34.6                           | 38.5   | .26    | 10.6    | 15.6           | 6.3             | .49      |
| F. F.                                                           | 8.64   | 8.95   | 5.8             | 7.87                           | 9.49   | 8.31   | 7.17    | 6.78           | 5.05            | 8.9      |
| Item "In" or "Out" on properties shown, as a self-felting fiber | K.F.   | In     | K.E.            | In                             | In     | C. M.  | K.F.    | { C. M. K.F. } | In              |          |
| Item "In" or "Out" for adhesive mats                            | In     | In     | { C. M. F. F. } | In                             | In     | C. M.  | In      | C. M.          | { C. M. F. F. } | In       |

In Table III, the item 10 is chemically treated fiber identified as sample S-218-11.

The invention contemplates the production of fiber with control of particle size distribution, and subsequent treatment and use of the resulting fiber for the ultimate purpose of providing loosely felted masses having insulation efficiency, wherein properties of the fiber to form the felts, and properties of the felt are predetermined by the coarseness modulus and other properties.

Fig. 3 shows diagrammatically the relation of the original fiber to the subsequent uses. Generally, and practically the fiber may be provided in dry or moist bulk, dry compacts such as bales and dry laps, and moist compacts, such as bales and wet lap. These are forms of convenience from which ultimate felts may be made. Bulk fiber, either dry or moist may be assembled to form ultimate mats or other masses at controlled densities. Compacts, moist or dry, may be fluffed or disintegrated, to reproduce a bulk form.

Dry bulk fiber may be assembled into a self-felted insulating body by mechanical packing, pneumatic conveyance and deposition from air currents as described in Heritage U. S. Serial No. 294,212, filed September 9, 1939, or other methods.

Wet felting comprises assembling wet or moist fibers with or without adhesive, to form mats. Felting from water suspension may be done under conditions to avoid forming dense mats. The foaming process of Bryant U. S. No. 1,821,856 is one such method.

Fig. 3 is a diagram showing the courses fibers may take in the formation ultimately of loosely felted bodies, such as insulation mats. The block 20 represents a process of producing fiber of coarseness modulus desired. Lines 21, 22, and 23, indicate respectively the paths to direct felting, direct drying, and addition of water. Along path 21, there are represented felting 24 with or without adhesive while moist from the grinding, and drying 25.

Along path 22, the fiber may be baled at 26 directly from the grinding, followed by fluffing 27, then felting moist at 28 and drying 29. Also the fluffed fiber 27 may be first dried at 30 and dry felted at 31 with or without adhesive.

On line 22 (direct drying) the dried fiber 23 may be felted at 32 with or without adhesive, or be baled dry at 33. After such baling it may be fluffed at 34, and then either dry felted at 35 with or without adhesive, or moist felted at 36 with or without adhesive, and dried at 37.

On path 23, water may be added, or the fibers suspended in water, in which case a fiber re-

39, then fluffed at 40. The dry fluffed fiber may be dry felted at 41 with or without adhesive, or wet felted at 42 with or without adhesive and dried at 43. Instead of drying the recovered fiber from filtration 38, it may in the so-called "filtering" be obtained as a wet-lap, like paper pulp, as at 44. This may be dried at 45, or fluffed wet as at 46, or dried at 45 and rewetted and fluffed wet (46). The dry lap 45 may be dry fluffed at 47, and dry felted at 48 with or without adhesive, or wet felted at 49 and dried at 50. The wet fluffed fiber 46 may be wet felted at 51 with or without adhesive and dried at 52, or the wet fluff 46 may be dried at 53 and dry-felting at 54 with or without adhesive.

It is to be understood that various treating agents or other fibers may be added, and that any method of felting is permitted.

The series of Table I represents fibers not treated. A treatment of the fibers as by sizing or impregnating, may not change the coarseness modulus, but it may so alter the fibers that other measurable and important properties change. Table IV shows examples of green jack pine fiber untreated and treated with rubber latex to reduce the dustiness of it, and to improve its qualities for pneumatic felting, or with other materials. This illustrates fibers of the same coarseness modulus, but of different evaluation.

Table IV

| Sample             | .9% latex solids | 202-47 | 202-46 |
|--------------------|------------------|--------|--------|
| Treatment          |                  | None   |        |
| Coarseness modulus |                  | 198    | 198    |
| Free-footage       |                  | 9.2    | 9.5    |
| M.E.               |                  | .333   | .327   |
| K.F.               |                  | 100    | 123    |
| M.F.               |                  | .257   | .266   |
| K.E.               |                  | 31     | 49     |
| Impact resistance  |                  | 3.7    | 4.1    |
| K-value            |                  | .232   | .228   |
| Dust percent       |                  | 1.0    | 2.8    |

From many determinations it has been ascertained that for insulating self-felted fibrous bodies the fibers used should have properties within the following limits.

| Property                 | Minim-<br>um | Maxi-<br>mum |
|--------------------------|--------------|--------------|
| Free-footage             | 6.0          | None         |
| Specific felting K.F.    | 20           | 80           |
| Specific elasticity K.E. | 50           | None         |
| Coarseness modulus       | 60           | 250          |

For adhesively bound mats, the elastic and felting qualities need not meet the above limitations.

Given fibers within these limits the K-value

will be satisfactory, the mechanical working properties will be satisfactory for one or more methods, and the stability of the insulating mat particularly against settling when the mat lacks adhesive, will be assured, if it is formed in accordance with the evaluation of the fiber. The formation must observe the impact resistance in order to employ a non-settling density, which will vary according to the conditions to which the mat will be subjected. A density between 3 and 4 pounds per cu. ft. is usual for these dry felted unbound fibers.

It is generally known with respect to fibrous insulating mats that as the density increases or decreases from some particular density, the K-value rises. For the fiber of the present invention when used in self-felted mats, it has been found that as a general rule the K-value is not above .25, when the density of the mat is within the range from 2 to 6 pounds per cu. ft. Where the C. M. is from 100 to 250, the said density may be anywhere in the range from 2 to 6, but for fiber having a C. M. of below about 100, the density must be nearer the middle of the range to assure the desired K-value of not over .25.

#### FIBER CLASSIFIER

In order that the coarseness modulus may be determined as it is herein defined and used, the apparatus is set forth in Figs. 4 to 8.

A base 60 has uprights 61 supporting a table 62, which table presents two upright guides 63 and 64 for a sliding cross-head 66. The table also supports a vertical cylinder 67, of 5½ inches inside diameter, open at the top 68 and capped at the bottom 69 where an outlet pipe 71 is connected. In the cylinder, a plunger operates. It comprises a plunger rod in the form of a water-conduit 72, carrying three piston-heads 73, 74 and 76 which provide perforations for filtering fiber. The plunger-pipe 72 has a telescopic water-connection with a fixed water-pipe 77 located at the top of the guides 63—64, and said fixed pipe connects by line 78 to a pressure controlled water supply line 79. A valve 81 and pressure gauge 82 indicate the controls of the water supply to the plunger. Also a water-supply connection 83 with valve 84 leads to the lower capped end 69 of the cylinder, whereby the cylinder may be filled with water. A valve 86 in the cylinder drain-line 71 controls the outflow in line 87 which discharges into a waste-funnel 89 over which is placed a fiber collecting screen 91 of 80 mesh. (U. S. Standard 8019.)

The cross-head 66 is balanced by counter-weights 92 over pulleys 93, and the parts are so arranged that the cross-head may be raised to bring the plunger and its lower perforated head 76 outside of the cylinder 67. In normal operation the plunger rides in the cylinder in the position shown, with a stroke of 3 inches from a rotary drive operating at 65 R. P. M. This drive comprises a motor 92, a gear box 93, and two crank pins 94. From the crank pins 94 there are connecting rods 96 to the cross-head 66, where a detachable union 97 is provided, for removal of the driving rods for raising the cross-head.

The pistons 73, 74 and 76 have top areas of 4½ inches diameter. In piston 73, this area has holes 98 (Fig. 6) which are  $\frac{1}{16}$  inch in diameter and arranged at a uniform spacing of 100 per sq. in. In piston 74 (Fig. 7) there are holes 99 which are  $\frac{3}{64}$  inch in diameter and arranged at a uniform spacing of 144 per sq. in. In piston 76 (Fig. 8) there is a wire screen 101 of 32 meshes per inch.

In addition, above each piston head there are two short nozzles 102 for water-jets. These are at an angle from the vertical of 45° and offset  $\frac{1}{4}$  inch from a diametrical line. The nozzles directly above each piston head have  $\frac{3}{16}$  inch diameter openings. In addition there is an extra set of nozzles 103 top-most to lie above the top piston and their openings are  $\frac{1}{16}$  inch in diameter. Water pressure of 25 to 30 pounds at gauge 82 forces jets through the nozzles to give a rotary swirl to fibers on the perforated plates or screens.

The top-plate 88 operates at a level of 8½ to 11½ inches from the top rim of cylinder 67; and the two lower perforated members are respectively 6 and 12 inches below plate 98.

In operation to determine coarseness modulus, the cylinder is filled by operating valve 84, until the water-level is 1 inch from the top. Then the motor is started, and valves 86 and 81 opened, whereby water enters and drains away, the adjustments being such as to maintain the original water level in the cylinder. Then a weighed sample of fiber, with known dry weight, for example about 5 grams, is placed in the cylinder above the top piston. The fibers thus become separated according to size, as the machine is operated for 15 minutes. Then the water is drained from the cylinder, and the fibers on the plates or screens are collected, oven-dried, or dried in a steam press, and weighed, giving 4 fractions for use in determining the coarseness modulus. The difference passing screen 91 is merely recorded as the past 4th fraction.

#### FRACTIONATED FIBER

A mass of jack pine fiber A (see Table VI) evaluating with suitable characteristics for a self-felting fiber has been treated by a suitable process of dry fractionation whereby it is split into a coarse fraction C and a fine fraction F. Then the coarse fraction is again similarly divided producing a coarse fraction CC and a fine fraction CF. These masses of fiber evaluate as follows:

Table VI

| Property                                                | A Composite | C Coarse from A | F Fine from A | CC Coarse from C | CF Fine from C |
|---------------------------------------------------------|-------------|-----------------|---------------|------------------|----------------|
| Free-footage—F. F.                                      | 9.75        | 9.80            | 9.45          | 9.22             | 9.00           |
| K <sub>E</sub>                                          | 141         | 150             | 133           | 110              | 115            |
| M <sub>E</sub>                                          | .328        | .332            | .338          | .333             | .357           |
| K <sub>F</sub>                                          | 47          | 34              | 42            | 23               | 36             |
| M <sub>F</sub>                                          | .253        | .250            | .256          | .203             | .266           |
| Fraction No.—                                           |             |                 |               |                  |                |
| 1                                                       | 18.0        | 38.2            | 2.8           | 53.6             | 11.8           |
| 2                                                       | 12.8        | 14.4            | 19.2          | 14.0             | 25.2           |
| 3                                                       | 27.6        | 20.2            | 35.0          | 16.0             | 33.2           |
| 4                                                       | 23.2        | 14.4            | 25.0          | 6.2              | 16.2           |
| 4+                                                      | 18.4        | 12.8            | 18.0          | 10.2             | 13.6           |
| Coarseness modulus—                                     |             |                 |               |                  |                |
| C.M.                                                    | 188.8       | 250             | 163.8         | 294.6            | 205.4          |
| K-value                                                 | .227        | .222            | .224          | .241             | .232           |
| "In" or "Out" on property shown, for self-felting fiber | In          | (1)             | In            | CM               | In             |

<sup>1</sup> "In" but at limit on CM.

When fibers are fractionated a different set of laws appears to hold with respect to the resulting K-value as related to the CM from the fibers and the density of the mat.

The above table confirms the fact that high coarseness modulus produces high K, yet it shows that the presence of the coarser particles mixed with fines as in the composite is permitted. It shows also that with very little change in free-footage or fluffiness, there may be wide variations in the particle size distribution, and in thermal efficiency in self-felted mats at 3.8 pounds per cu.

ft. It follows that no one property may be used as a direct indication of the thermal efficiency. These particular results show that any judgment evaluation of any one fiber on the basis of "fluffiness" (free-footage) is not a completely reliable indication of its utility as a thermal insulating fiber.

#### ADHESIVELY BOUND MAT

The bulk fiber may be adhesively bound to form flexible insulating blankets of high thermal efficiency. Thus, rough green jack pine is reduced to fiber using a fire-retarding agent with the chips entering an Asplund machine, in accordance with the applications of Heritage and Walter, Serial No. 332,682, and Serial No. 332,683, both filed May 1, 1940. Thus, for 100 pounds of dry wood are used 8 pounds of ammonium sulfate and .08 pound of calcium carbonate. The machine is adjusted and operated to give fiber of the desired characteristics. The discharged fiber is exemplified by reference to one having the following characteristics:

|                                       |                  |
|---------------------------------------|------------------|
| Free-footage                          | 8.3              |
| Specific elasticity (K <sub>E</sub> ) | 97               |
| Absolute elasticity (M <sub>E</sub> ) | .400             |
| Specific felting (K <sub>F</sub> )    | 34               |
| Absolute felting (M <sub>F</sub> )    | .291             |
| K-value                               | .241             |
| Impact resistance                     | <sup>1</sup> 3.1 |

<sup>1</sup> (In board-feet per pound, or 3.88 in pounds per cu. ft.)

#### Particle size distribution:

|                    |       |
|--------------------|-------|
| 1st fraction       | 4.2   |
| 2nd fraction       | 17.4  |
| 3rd fraction       | 22.0  |
| 4th fraction       | 28.4  |
| 4+ fraction        | 28.0  |
| Coarseness modulus | 141.4 |

The discharged fiber has about 100 pounds of water per 100 pounds of dry wood, the mass being moist fibers not felted. These may be felted moist by suitable process, but since aqueous binder is added to effect union of the felt, the fibers are partially dried so that the formed mat will not be too wet. They are dried to have 20 to 30 parts of water per 100 parts of dry fiber substance.

The fibers are deposited from air suspension to form a mat, preferably by gravity showering the fibers onto a moving belt. As the fibers fall they pass through a fine spray of liquid binder, then on the screen they pile up into a loose felt. This is dried and the binder unites the fibers in the felt.

The adhesive may be of many types. A liquid may have adhesive and other agents in it, for example a water-proofing size, and mould-proofing agents, insecticides and the like. An aqueous starch solution at about 2.5% has been successfully used. Such a solution having also about .5% of other materials, such as wax in emulsion form, and insecticide.

Such a mat made at 1 inch thickness, may have by weight about 120 to 140 parts of fiber, 20 parts of starch, about 15 parts of fire-proofing agent, about 2 to 4 parts of wax, and about 6 to 8 parts of preservative, per 1000 sq. ft. It has a K-value of about .235. Such a mat may be placed between paper liners, asphalted, plain, flat or creped, in varying combinations to provide flexible blanket insulation.

#### SELF-FELTED MATS

The mere compression of fiber to a mat pro-

duces felting, and such mats are hereinabove indicated as having been so made, where the K-value is given. It has been determined that frames with mats of the same density, packed either by machine, by hand, or by a pneumatic process as above referred to, have identical K-values, where the fiber is the same, and where the arrangement is heterogeneous, and the mat substantially uniform in density.

10 It is of course understood that some fibers within the scope of the present invention are so far from the border lines of efficiency that they are capable of dilution with other fibers without bringing the mixture outside of the bounds of the present invention.

15 The foregoing description and explanation shows that the invention may be practiced in many ways differing from the specific illustrations given, without departing from the spirit and scope of the invention as expressed in the appended claims.

I claim:

1. Thermal insulation material comprising an aggregate mass of fibers the composition of which is essentially lignocellulose, said fibers being characterized by a coarseness modulus within the range from 60 to 250, and further characterized when dry and in substantially unfelted mass formation by a free-footage not less than 6 board-feet per pound; by a specific felting resistance within the range of 20 to 80 pounds per sq. ft. at a density corresponding to 3.15 board-feet per pound; and by a specific elasticity of not less than 50 pounds per sq. ft. at a density corresponding to 3.15 board-feet per pound.

2. A fiber mass according to claim 1 in which the fibers are derived from long-fibered wood, characterized by a coarseness modulus within the range from 130 to 250.

3. A fiber mass according to claim 1 in which the fibers are derived from short-fibered wood, characterized by a coarseness modulus within the range from 60 to 160.

4. Thermal insulation comprising felted fiber mat having fibers of lignocellulose material entangled and bound together by the natural felting property of the fiber, said mat having a density not in excess of 4 pounds of fiber per cu. ft., said fibers having the characteristics of the fiber of claim 1.

5. Thermal insulation comprising felted fiber mat having fibers of lignocellulose material entangled in felt formation and adhesively united, said mat having a density not in excess of 4 pounds of fiber per cu. ft., said fiber having the characteristics of the fiber of claim 1.

6. Thermal insulation material comprising an aggregate mass of fibers the composition of which is essentially lignocellulose, said fibers having at the surface a small quantity of an added agent imparting water-resistance to the fibers, said agent being selected from the group consisting of bituminous asphalt and of solids of rubber latex, said fibers being characterized by a coarseness modulus within the range from 60 to 250, and further characterized when dry and in substantially unfelted mass formation by a free-footage not less than 6 board-feet per pound; by a specific felting resistance within the range of 20 to 80 pounds per sq. ft. at a density corresponding to 3.15 board-feet per pound; and by a specific elasticity of not less than 50 pounds per sq. ft. at a density corresponding to 3.15 board-feet per pound.

7. Thermal insulation material comprising an

aggregate mass of fibers the composition of which is essentially lignocellulose, said fibers having at the surface a small quantity of the solids of rubber latex, said fibers being characterized by a coarseness modulus within the range from 60 to 250, and further characterized when dry and in substantially unfeated mass formation by a free-footage not less than 6 board-feet per pound; by a specific felting resistance within the range of 20 to 80 pounds per sq. ft. at a density corresponding to 3.15 board-feet per pound; and by a specific elasticity of not less than 50 pounds per sq. ft. at a density corresponding to 3.15 board-feet per pound.

8. Thermal insulation material comprising an 15

aggregate mass of fibers the composition of which is essentially lignocellulose, said fibers having at the surface a small quantity of bituminous asphalt, said fibers being characterized by a coarseness modulus within the range from 60 to 250, and further characterized when dry and in substantially unfeated mass formation by a free-footage not less than 6 board-feet per pound; by a specific felting resistance within the range of 20 to 80 pounds per sq. ft. at a density corresponding to 3.15 board-feet per pound; and by a specific elasticity of not less than 50 pounds per sq. ft. at a density corresponding to 3.15 board-feet per pound.

CLARK C. HERITAGE.

CERTIFICATE OF CORRECTION.

Patent No. 2,325,055.

July 27, 1943.

CLARK C. HERITAGE.

It is hereby certified that error appears in the printed specification of the above numbered patent requiring correction as follows: Page 5, second column, line 57, for "(M<sub>A</sub>)" read --(M<sub>E</sub>)--; line 58, for "(M-)" read --(M<sub>F</sub>)--; page 11, second column, line 72, for "pes" read --per--; and that the said Letters Patent should be read with this correction therein that the same may conform to the record of the case in the Patent Office.

Signed and sealed this 14th day of September, A. D. 1943.

Henry Van Arsdale,  
(Seal) Acting Commissioner of Patents.